

[54] ORTHO ALKYL PHENOL AND ORTHO  
ALKYL PHENOL SULPHIDE LUBRICATING  
OIL ADDITIVES

[75] Inventors: Phillip William Brewster, Wyoming, Canada; Peter Collen Hamblin, Cheadle; James Pennycook Rutherford, Abingdon, both of England

[73] Assignee: Exxon Research &amp; Engineering Co., Linden, N.J.

[22] Filed: Sept. 5, 1974

[21] Appl. No.: 503,370

## Related U.S. Application Data

[63] Continuation-in-part of Ser. No. 417,121, Nov. 11, 1973.

## [30] Foreign Application Priority Data

Sept. 7, 1973 United Kingdom..... 1980/73  
May 23, 1974 United Kingdom..... 23068/74[52] U.S. Cl. .... 252/48.2; 44/76; 44/78;  
252/52; 252/393; 252/404[51] Int. Cl. 2. C10M 1/38; C10M 3/32; C10M 5/28;  
C10M 7/36[58] Field of Search ..... 44/76, 78; 252/48.2, 52,  
252/493, 404

## [56] References Cited

## UNITED STATES PATENTS

|           |         |                      |        |
|-----------|---------|----------------------|--------|
| 2,237,627 | 4/1941  | Olin .....           | 260/60 |
| 3,250,712 | 5/1966  | Coffield .....       | 252/48 |
| 3,647,885 | 3/1972  | Geering et al. ....  | 260/60 |
| 3,745,117 | 7/1973  | Fujisawa et al. .... | 252/48 |
| 3,844,964 | 10/1974 | Kennedy .....        | 252/48 |

Primary Examiner—Delbert E. Gantz

Assistant Examiner—I. Vaughn

Attorney, Agent, or Firm—Frank T. Johmann

## [57] ABSTRACT

An additive mixture for lubricating oils and fuel oil having good antioxidant and anticorrosion properties comprising: (a) 45-75 wt.% of an ortho alkyl phenol; (b) 5-20 wt.% of an ortho alkyl phenol disulphide and (c) 15-40 wt.% of an ortho alkyl phenol trisulphide. Optionally the additive may also contain small amounts of the corresponding mono- and tetrasulphide. Such additives may be made by reacting an alkyl phenol with sulphur in the presence of an organic amine having a  $pK_b$  of between 2 and 12, e.g. morpholine.

16 Claims, No Drawings

ORTHO ALKYL PHENOL AND ORTHO ALKYL  
PHENOL SULPHIDE LUBRICATING OIL  
ADDITIVES

This invention relates to additives which act as antioxidant and anti-corrosion additives in lubricating oils.

This application is a continuation-in-part of our prior filed application Ser. No. 417,121 filed Nov. 19th, 1973.

It has been found that certain mixtures of hydrocarbyl substituted phenols and sulphurised hydrocarbyl substituted phenols have very good antioxidant and anti-corrosion properties when added to lubricating oils.

According to this invention an additive mixture suitable for addition to lubricating oils and fuel oils comprises (a) 45-75 wt.% of a phenol substituted with one or two hydrocarbyl groups, one of which must be in the ortho position, (b) 5-20 wt.% of a hydrocarbyl substituted phenol disulphide, each benzene ring having one or two hydrocarbyl substituents, one of which in each ring being in the ortho position with respect to the hydroxyl group and (c) 15-40 wt.% of a hydrocarbyl substituted phenol trisulphide, each benzene ring having one or two hydrocarbyl substituents, one of which in each ring being in the ortho position with respect to the hydroxyl group.

Optionally the additive also contains not more than 10% by weight of the other three components, of (d) a hydrocarbyl substituted phenol tetrasulphide, each benzene ring having one or two hydrocarbyl substituents, one of which in each ring being in the ortho position with respect to the hydroxyl group. Also the additive may contain not more than 5% by weight of the three components (a), (b) and (c), of (e) a hydrocarbyl substituted phenol monosulphide, each benzene ring having one or two hydrocarbyl substituents, one of which in each ring being in the ortho position with respect to the hydroxyl group.

In components (a), (b), (c), (d) and (e) the hydrocarbyl substituents are preferably in aliphatic group, e.g. alkyl, cycloalkyl or alkenyl. If desired these substituents may be aromatic such as aryl, aralkyl or alkaryl, e.g. tolyl, phenylethyl or phenyl butyl.

It is preferred that the or each aliphatic group has at least 3 carbon atoms, e.g. from 4 to 20 carbon atoms. Examples are t-butyl, sec-butyl, amyl, hexyl, cyclohexyl, octyl, isoctyl, nonyl, decyl, dodecyl, octadecyl or eicosyl groups. It is preferred that the alkyl groups be branched, and especially tertiary alkyl groups such as t-butyl, t-octyl and t-dodecyl.

Other aliphatic groups which are suitable are those derived from the polymerization of a mono olefin, i.e. an alkenyl group. Suitable olefins are, for example, ethylene, propylene, butylene, 1-hexylene, etc. Such alkenyl groups usually contain from 20 to 500 carbon atoms, e.g. from 60 to 70 carbon atoms.

For each component (a) to (e) there may be one or two hydrocarbyl groups per benzene ring, provided one of them is in the ortho position with respect to the hydroxyl group. When there are two hydrocarbyl groups per benzene ring it is preferred that both of the hydrocarbyl groups are in the ortho position with respect to the hydroxyl group, but one of them may, of course, be in another position i.e. meta or para with respect to the hydroxyl group.

It is to be understood that the hydrocarbyl group may be the same or different both for each separate component and as between the separate components. Generally, however, the hydrocarbyl groups will be the same for components (a), (b) and (c) and for components (d) and (e) if present. Usually the number of hydrocarbyl groups per benzene ring will be the same for all components and if there are two for each component usually they will all be in the same position with respect to the hydroxyl group.

For components (b), (c), (d) and (e) the sulphur linkage between the two benzene rings may be in the ortho but is preferably in the para position with respect to the hydroxyl group.

Usually components (b), (c), (d) and (e) can be represented by the formulae:



where R is a hydrocarbyl group, preferably alkyl, which may be different in one or more cases, but is usually the same; and wherein x for components (b), (c), (d) and (e) is respectively 2, 3, 4 and 1.

The preferred proportions for components (a), (b) and (c) are respectively 55-65 wt.%, 10-15 wt.% and 20-35 wt.%. Typical proportions for components (d) and (e) are respectively 3-7 wt.% and 1-2 wt.%, based on the weight of components (a), (b) and (c).

Thus, in a typical additive wherein component (a) is 2, 6, di-tert butyl phenol and the other components (b), (c), (d) and (e) are the corresponding 2, 6, di-tert butyl phenol sulphides there is

- about 62 wt.% of component (a)
- about 12 wt.% of component (b)
- about 19 wt.% of component (c)
- about 5 wt.% of component (d) and
- about 2 wt.% of component (e)

The additive can be made by mixing together individual components or by a novel method according to this invention.

It is known to produce sulphurised alkyl phenols by reacting an alkyl phenol with sulphur mono- or di-chloride, but such products tend to cause copper corrosion probably due to the presence of corrosive sulphur species e.g. sulphochlorinated alkyl phenol.

Attempts have been made to avoid the presence of chlorine by sulphurising an alkyl phenol by sulphur alone; but this has not been possible since the reactant is highly unreactive. We have not surprisingly found a method of preparing sulphurised alkyl phenols using sulphur as the sulphurising agent.

According to this invention sulphurised alkyl phenols are prepared by a process in which an alkyl phenol of the formula



where R is an aliphatic group (e.g. an alkyl or cycloalkyl group) and m and n are integers of from 1 to 6 inclusive provided m plus n is not more than 6, is reacted with sulphur in the presence of an organic amine having a pK<sub>a</sub> of between 2 and 12.

2 alkyl phenols which may be used have the for-



3 d n being integers of from 1 to 5. Preferred alkyl 10 oils are those where m and n are both 1, but alkyl 15 roxy benzenes (m = 2) and dialkyl phenols (n = 2) are quite suitable. It is to be understood that when n 20 or more each alkyl group R can be different if desired. It is preferable that the or each aliphatic (alkyl 25 cycloalkyl) group R, has at least 3 carbon atoms e.g. 30 6 to 20 carbon atoms. Examples are t-butyl, s-, amyl, hexyl, cyclohexyl, octyl, isoctyl, nonyl, dodecyl, octadecyl or eicosyl groups.

Instead of using an alkyl or cycloalkyl phenol it is 35 possible to use other phenols having the same general 40 structure where the group R is an aliphatic group, e.g. derived from the polymerization of a mono-olefin, an alkenyl group. Suitable olefins are for example, 45 ethylene, propylene, butylene, 1-hexylene etc. Such 50 vinyl groups usually contain from 20 to 500 carbon atoms, e.g. from 60 to 70 carbon atoms.

55 The amine which is used must have a  $pK_b$  of between 12, and it is preferred that it has a  $pK_b$  of between 10.  $pK_b$  is the negative logarithm (to base 10) of 60 the equilibrium constant  $K_b$  of the reaction of the base with water. Thus, for the reaction



$$= \frac{[BH^+] [OH^-]}{[B]}$$

65 The primary amines include Primene 81-R (a 70 tri-alkyl primary amine containing 12-14 carbon atoms —  $pK_b \approx 4.2$ ) and the 2-, 3- and 4-amino pyridines ( $pK_b = 7.1$ , 7.9 and 4.8 respectively). Suitable 75 secondary amines include pyrrolidine ( $pK_b = 2.73$ ), azine ( $pK_b = 4.19$ ), piperidine ( $pK_b = 2.80$ ), morpholine ( $pK_b = 5.67$ ), pyrid-4-one ( $pK_b = 10.70$ ), imidazole ( $pK_b = 7.00$ ), pyrazole ( $pK_b = 11.5$ ) and di-n-amine ( $pK_b = 2.72$ ). Tertiary amines which can be 80 included are pyridine ( $pK_b = 8.86$ ), the 2-, 3- and 4-yl pyridines ( $pK_b = 8.0$ , 8.3 and 8.0 respectively), 85 imidazole ( $pK_b = 10.69$ ), cinnoline ( $pK_b = 11.36$ ), azine ( $pK_b = 11.90$ ), quinoline ( $pK_b = 9.15$ ), isoquinoline ( $pK_b = 8.86$ ) and acridine ( $pK_b = 8.40$ ). Preferred amines are heterocyclic compounds having a 90 amino group, especially a secondary amino group. Particularly preferred secondary amines are piperidine and morpholine. Very suitable secondary amines are which are liquid at ambient temperatures.

95 The mole ratio of alkyl phenol to sulphur can vary, from about 2:1 to about 1:2. The amounts of amine are small, e.g. 0.1 to 10 wt.%, especially from 1 to 100 % based on the weight of alkyl phenol and sulphur.

105 The sulphurised alkyl phenol is preferably prepared by heating with stirring the alkyl phenol, flowers of sulphur and secondary amine. The temperature to which the mixture is heated may be from 100° to 150°, e.g. 150°C. The reaction mixture is preferably maintained at this temperature with stirring for a sufficient time e.g. about 45 minutes. After being maintained at this temperature the reaction mixture is then heated to a higher temperature e.g. 170° to 190°C pref-

110 erably 180°C, and held at this higher temperature for a period of time, e.g. 8 to 12 hours, preferably 10 hours. After being held at this higher temperature, the reaction mixture should be blown with nitrogen e.g. for about 2 hours.

115 As an even better method the alkyl phenol and sulphur may first be heated with stirring, e.g. to 120°C, and then the secondary amine added.

120 In order to minimise or prevent solids formation by sublimation in the cold parts of the reactor, the solids being unreacted phenol and a reaction product between sulphur and the amine, it has been found advantageous to use an alcohol as a solvent when reacting the alkyl phenol with sulphur in the presence of the amine. 125 Particularly suitable alcohols include n-butanol, amyl alcohol, isoheptanol and other alcohols having boiling points less than 180°C.

130 The amount of alcohol used as solvent can vary greatly but amounts of between 5 and 25 wt.% e.g. about 15 wt.%, based on the weight of alkyl phenol, sulphur and amine have been found to be suitable.

135 Usually the additive mixture contains a diluent oil which may, for example, be any mineral lubricating oil. Other suitable diluent oils include synthetic ester lubricating oils. When making the additive mixture by the novel method described above the starting alkyl phenol is usually dissolved in the oil.

140 The amount of diluent oil can vary but usually the oil solution contains from 10 to 40 wt.% of oil, e.g. about 15-25 wt.% of oil.

145 The additive mixture can be added to a lubricating oil especially a crankcase lubricant, where it acts as an antioxidant and an anti-corrosion agent. It can also be added to a fuel oil, e.g. gasoline or diesel fuel, as a minor proportion by weight.

150 The lubricating oil may be any animal, vegetable or mineral oil, for example, petroleum oil fractions ranging from naphthas to spindle oil to SAE 30, 40 or 50 lubricating oil grades, castor oil, fish oils or oxidised mineral oil.

155 Suitable synthetic ester lubricating oils include diesters such as di-octyl adipate, dioctyl sebacate, didecyl azelate, tridecyl adipate, didecyl succinate, didecyl glutarate and mixtures thereof. Alternatively, the synthetic ester can be a polyester such as that prepared by reacting polyhydric alcohols such as trimethylol propane and pentaerythritol with monocarboxylic acids such as butyric acid, caproic acid, caprylic acid and pelargonic acid to give the corresponding tri- and tetraesters.

160 Also, complex esters may be used as base oils such as those formed by esterification reactions between a dicarboxylic acid, a glycol and an alcohol and/or a monocarboxylic acid.

165 The preferred quantity of sulphurised alkyl phenol added to the lubricating oil is between 0.01 and 10%, e.g. between 0.1 and 5% by weight based on the total weight of oil plus additive mixture.

170 Other additives, for example, dispersants (e.g. polybutene succinimides), VI improvers (e.g. vinyl acetate/fumarate copolymers), corrosion inhibitors (e.g. diol esters) or additional antioxidants (e.g. phenolic compounds) may be added to the lubricating oil.

#### EXAMPLE 1

175 An additive mixture was prepared which had the following composition:

|                        | wt.% |
|------------------------|------|
| Base oil diluent       | 23   |
| 2, 6-di-t butyl phenol | 42   |
| " monosulphide         | 1    |
| " disulphide           | 8    |
| " trisulphide          | 22   |
| " tetrasulphide        | 4    |

The additive mixture was tested in the Rotary Bomb Oxidation Test (RBOT) — ASTM D 2272 method — for its effect as an antioxidant in an oil. It was also tested as an anti-corrosion additive, using USA Federal Test Method Standard No. 791B Method 5321-1 (modified to run for 20 hours). For comparison purposes similar tests were carried out using 2, 6, di-t butyl phenol itself and the corresponding mono-, di-, tri- and tetra sulphides. Also tests were carried out on the oil alone which was a typical 10W/30 ashless mineral lubricating oil containing a VI improver and a dispersant. The results obtained were as follows:

It can be seen that the additive mixture shows superior properties both as an antioxidant and as an anti-corrosion agent.

## EXAMPLE 2

Sulphurised alkyl phenols were prepared by the following method.

- the alkyl phenol, sulphur, and piperidine were heated with stirring to 150°C and maintained at that temperature for 45 minutes.
- the temperature of the reaction mixture was then increased to 180°C and held for 90 minutes.
- the reaction mixture was then blown with nitrogen for two hours at 180°C.

The reaction details and results of ASTM D-130 copper corrosion tests are given below. For comparison an alkyl phenol was sulphurised with sulphur but in the absence of a sulphur-free secondary amine.

| Alkyl Phenol (AP)   | Mol. ratio AP:Sulphur | Amine      | Amine wt.% of reactant charge | S Content wt.%(a) | Free AP wt.%(a) | Cu Corrosion ASTM D-130(b) |
|---------------------|-----------------------|------------|-------------------------------|-------------------|-----------------|----------------------------|
| Mixed nonyl/dinonyl | 1.0:0.56              | Nil        | —                             | 1.39              | —               | 4c                         |
| "                   | 1.0:0.56              | Piperidine | 1.6                           | 3.37              | 41              | <1                         |
| "                   | 1.0:0.84              | "          | 2.0                           | 5.27              | 35              | 1b                         |
| Dodecyl             | 1.0:1.0               | "          | 2.0                           | 5.54              | 33              | 2a                         |
| "                   | 1.0:1.0               | "          | 6.0                           | 3.25              | 35              | <1                         |

(a)determined by liquid chromatography

(b)2.5 wt.% in mineral base oil having a viscosity of 150 S.S.U. at 100°F.

## RBOT

| Additive       | Treat level (wt. 5) | Induction Period (minutes) |     |
|----------------|---------------------|----------------------------|-----|
|                |                     | 80                         | 114 |
| Mixture phenol | 1.5*                | 80                         | 40  |
| monosulphide   | 1.5                 | 114                        |     |
| disulphide     | 1.55                | 67                         |     |
| trisulphide    | 0.78                | 61                         |     |
| tetrasulphide  | 0.56                | 54                         |     |
| None           | 0.44                | 50                         |     |
|                | —                   | 28                         |     |

\*including the 23 wt.% oil.

## Corrosion

| Additive      | Treat level (wt.%) | Wt. loss (mg/sq. in.) |      |
|---------------|--------------------|-----------------------|------|
|               |                    | Pb                    | Cu   |
| monosulphide  | 1.5*               | 2.6                   | 7.8  |
| disulphide    | 1.55               | 74.4                  | 6.2  |
| trisulphide   | 0.78               | 12.6                  | 2.4  |
| tetrasulphide | 0.56               | 1.0                   | 35.6 |
| None          | 0.44               | 0.6                   | 42.2 |
|               | —                  | 5000                  | —    |

\*including the 23 wt.% oil.

## EXAMPLE 3

Sulphurised alkyl phenols were prepared by heating with stirring to 120°C the alkyl phenol and sulphur. Morpholine was then added and the temperature of the mixture raised to 180°C with nitrogen sparging. When the level of H<sub>2</sub>S trapped in a caustic soda scrubber remained constant, usually after 5–15 hours, the temperature was reduced to 120°C and the mobile liquid was vacuum stripped at 150 mm Hg for 3–6 hours. In each case the product was diluted with a mineral base oil having a viscosity of 150 S.S.U at 100°F to 75% active ingredient.

The reaction details and results of ASTM D-130 copper corrosion tests are given below.

| Alkyl Phenol (AP) | Mol. ratio AP-Sulphur | Amine      | Amine wt.% of reactant charge | S(a) content wt.%(a) | Free(b) AP wt.%(b) | Product yield(c) % | Cu(d) Corrosion ASTM D-130 |
|-------------------|-----------------------|------------|-------------------------------|----------------------|--------------------|--------------------|----------------------------|
| Nonyl             | 1.0:1.0               | Morpholine | 4                             | —                    | —                  | 96                 | 2c                         |
| 2,6-di-t-butyl    | 1.0:1.0               | "          | 4                             | 7.1                  | —                  | 91                 | <1                         |
| ortho t-butyl     | 1.0:1.0               | "          | 4                             | —                    | 25                 | 89                 | 2c                         |
| 2,6-di-t-butyl    | 1.0:2.0               | "          | 4                             | 14.6                 | 15                 | 80                 | 4c                         |
| "                 | 1.0:1.0               | "          | 4                             | 6.6                  | 25                 | 82                 | 2c                         |

(a)Product diluted to 75% active ingredient with mineral lubricating oil having a viscosity of 150 S.S.U. at 100°F.

(b)Determined by thin layer chromatography

(c)Excluding free alkyl phenol.

(d)1.0 wt.% of diluted product (75% active ingredient) in mineral lubricating oil having a viscosity of 150 S.S.U. at 100°F.

## EXAMPLE 4

Sulphur and 2,6-di-tert butyl phenol (mole ratio S:phenol = 1:1) were heated with 4 wt.% based on the weight of sulphur and phenol, of piperidine for approximately 7 hours at 180°C with nitrogen sparging until the H<sub>2</sub>S evolved from the reaction was constant. (The H<sub>2</sub>S was trapped in NaOH scrubber and weighed periodically). The reaction product was diluted to 75 wt.% active ingredient with a mineral base oil.

| Mole Ratio<br>2,6-di-t-butylphenol:S | Antiwear Performance<br>Shell 4- ball wear Scar (mm) |
|--------------------------------------|------------------------------------------------------|
| (a) 1:1                              | 2.15                                                 |
| (b) 1:1.5                            | 1.80                                                 |
| (c) 1:2                              | 0.85                                                 |

Sulphurised alkyl phenols were added at 1.0 wt.% concentration to a mineral lubricating oil having a viscosity of 150 S.S.U. at 100°F.

The wear scar was determined after 1 hour at 60 kg load. The same oil having no additive gave a wear scar of 2.5 mm

## ANTIOXIDANT PERFORMANCE

A bearing corrosion rate described by Staudt et al. (SAE 680538) was used to evaluate the bearing weight loss and colour of Peter W1 bearings.

| Base Oil                                                           | BWL (mg) 36 hours at -140°C | Bearing Colour |
|--------------------------------------------------------------------|-----------------------------|----------------|
| No additive                                                        | 1810                        | Clean          |
| plus 1 wt.% sulphurised 2,6-di-t-butyl phenol (ratio as (b) above) | 2                           | Clean          |

The base oil contained a polyamine dispersant and ethylene propylene copolymer as VI improver to SAE 10W-30.

## EXAMPLE 5

10 moles (2060 g) of 2,6-di-tert butyl phenol, 10 mole (320 g) of flowers of sulphur and 372 g of isoheptanol were placed in a reactor and the temperature was raised to 120°C. 96 g (4 wt.% based on alkyl phenol plus sulphur) of morpholine was added. The temperature was raised to 180°C and maintained at this level for 20 hours with a nitrogen purge. 115 g of hydrogen sulphide was trapped out in a caustic soda scrubber. The solvent was removed by vacuum stripping and the temperature was raised to 90°C and a vacuum of 150 mm Hg absolute maintained until the exhaust gas from the vacuum pump did not discolour lead acetate paper, i.e. the product contained little hydrogen sulphide. The brown liquid product was diluted to 75% active ingredient (a.i.) with a 150 SSU lubricating oil and found to contain 6.4 wt.% sulphur.

## EXAMPLE 6

The procedure of Example 5 was repeated using 1075 g of Ethyl 733 (which is a mixture of mono-, di- and tri-t-butyl phenols in the ratio of about 15:75:10) instead of 2,6-di-tert butyl phenol, 160 g of sulphur, 25 g morpholine, 127 g of amyl alcohol instead of isoheptanol and a 7 hour reaction time at 180°C instead of a

20 hour reaction time. The 75 a.i. product contained 7.5 wt.% sulphur.

## EXAMPLE 7

Example 6 was repeated exactly only using about 140 g amyl alcohol and reacting at 180°C for 20 hours. The 75 wt.% a.i. product contained 6.4 wt.% sulphur.

## EXAMPLE 8

The procedure of Example 6 was used but using instead of amyl alcohol, 75.6 g of n-butanol. The 75 wt.% a.i. product contained 7.5 wt.% of sulphur.

What is claimed is:

1. An additive mixture comprising
  - a. 45-75 wt.% of a phenol substituted with one or two hydrocarbyl groups, one of which must be in the ortho position,
  - b. 5-20 wt.% of a hydrocarbyl substituted phenol disulphide, each benzene ring having one or two hydrocarbyl substituents, one of which in each ring being in the ortho position with respect to the hydroxyl group and
  - c. 15-40 wt.% of a hydrocarbyl substituted phenol trisulphide, each benzene ring having one or two hydrocarbyl substituents, one of which in each ring being in the ortho position with respect to the hydroxyl group.

2. An additive mixture according to claim 1 which also contains not more than 10% by weight based on the weight of components (a), (b) and (c), of (d) a hydrocarbyl substituted phenol tetrasulphide, each benzene ring having one or two hydrocarbyl substituents, one of which in each ring being in the ortho position with respect to the hydroxyl group.

3. An additive mixture according to claim 1 which also contains not more than 5% by weight based on the weight of the three components (a), (b) and (c), of (e) a hydrocarbyl substituted phenol monosulphide each benzene ring having one or two hydrocarbyl substituents, one of which in each ring being in the ortho position with respect to the hydroxyl group.

4. An additive mixture according to claim 1 wherein the hydrocarbyl substituents in the components are aliphatic groups.

5. An additive mixture according to claim 4 wherein the aliphatic groups are alkyl groups containing 4 to 20 carbon atoms.

6. An additive mixture according to claim 5 wherein the aliphatic group is a tertiary alkyl group.

7. An additive mixture according to claim 6 wherein the tertiary alkyl group is t-butyl, t-octyl or t-dodecyl.

8. An additive mixture according to claim 1 wherein there are two hydrocarbyl groups in the ortho position with respect to the hydroxyl group in each of the components.

9. An additive mixture according to claim 1 wherein the sulphur linkage in any sulphide is in the para position with respect to the hydroxyl group.

10. An additive mixture according to claim 3 which comprises a mixture of compounds each having the formula:



where R is an alkyl group and x is 1, 2, 3 or 4.

11. An additive mixture according to claim 1 which comprises 55-65 wt.% of component (a), 10-15 wt.% of component (b) and 20-35 wt.% of component (c).

12. An additive mixture comprising  
about 62 wt.% of 2, 6, di-tert butyl phenol,  
about 12 wt.% of 2, 6, di-tert butyl phenol disulphide,  
about 19 wt.% of 2, 6, di-tert butyl phenol trisulphide,  
about 5 wt.% of 2, 6, di-tert butyl phenol tetrasulphide, and  
about 2 wt.% of 2, 6, di-tert butyl phenol monosulphide.

13. An oil solution comprising 10 to 40 wt.% of diluent oil and 60 to 90 wt.% of the additive mixture according to claim 1.

14. A lubricating oil composition comprising a lubricating oil and 0.01 to 10 wt.% of the additive mixture according to claim 11.

15. A lubricating oil composition comprising a major proportion by weight of a lubricating oil and a minor proportion by weight of the alkyl phenol additive mixture according to claim 1.

16. A lubricating oil composition comprising a major proportion by weight of a lubricating oil and a minor proportion by weight of the additive mixture of alkyl phenols according to claim 12.

\* \* \* \* \*